

## UNITED STATES PATENT OFFICE

2,527,476

## CYANOACETYLHYDRAZONES AS PHOTOGRAPHIC COLOR COUPLERS

Pierre Joseph Marie Bruylants, Winksele-Veltem, near Louvain, and Philibert Leopold Jozef Raymond Merckx, Mortsel, near Antwerp, Belgium, assignors to Gevaert Photo-Producten N. V., Mortsel-Antwerp, Belgium, a company of Belgium

No Drawing. Application March 14, 1947, Serial No. 734,854. In Germany March 17, 1941

Section 1, Public Law 690, August 8, 1946  
Patent expires March 17, 1961

11 Claims. (Cl. 95—6)

1

This invention relates to photographic color developers and to processes for color development applicable in color photography.

It is known that colored photographs may be obtained by using a developer which during the development forms colored insoluble oxidation products. These products color the gelatine around the silver grains of the silver image.

It is also known to obtain colored images by using in the developing baths certain substances called color couplers which combine with the oxidation products of the developer with the formation of dyestuffs which precipitate simultaneously with the developed silver grains.

Many color couplers have hitherto been used or proposed, such as substituted or unsubstituted phenols and naphthols, nitrophenylacetonitriles and acetamide derivatives, characterized by the presence of an acid-reactive methylene group, isoxazolones, coumarones and pyrazolones.

Up to now, no theory has been advanced for the mechanism of photographic color development. Consequently, it is impossible to specify in advance with dependable certitude whether a given product is a usable color coupler or not.

Furthermore, although numerous color couplers are known, it is not always possible to choose among them the product which will give by condensation with the oxidation product of the developer the desired color corresponding to the tint of the dyestuffs already formed or subsequently to be formed in other layers. A further limitation in connection with the color couplers already known resides in the fact that only such color couplers can be used which form dyestuffs which are both non-diffusing in water and stable to photographic baths.

The present invention relates to a new group of color couplers which meet the aforesaid conditions.

Cyanoacetylhydrazide can scarcely be considered as a usable color coupler. If added to a developer which contains among others diethyl para-phenylenediamine, it only gives a slightly colored image.

Unexpectedly, we now have found that very favorable results as to color intensity and color brightness are obtained by adding to the developers as color couplers mono- or polycyanoacetylhydrazones derived from substances without a reactive methylene group.

These mono- and polycyanoacetylhydrazones are obtained by condensation of one or more cyanoacetylhydrazide molecules with products containing one or more groups which may react

with the NH<sub>2</sub> group of the hydrazides, such as aldehydes, ketones, dialdehydes, diketones, keto-aldehydes, and halogen compounds containing the group —CX<sub>2</sub> wherein X represents an halogen atom such as CH<sub>3</sub>—CO—CHCl<sub>2</sub> and



15 Color couplers obtained by condensation of cyanoacetylhydrazides with products containing one or more reactive methylene groups have been described in U. S. Patent 2,375,344 and are not included in the present invention.

20 As typical examples of color couplers of the new group, the following may be mentioned:



25 Cyanoacetylhydrazone of vanillin



30 Cyanoacetylhydrazone of piperonal



35 Cyanoacetylhydrazone of phenylacetaldehyde



40 Cyanoacetylhydrazone of crotonaldehyde



45 Cyanoacetylhydrazone of beta-furylacrolein



50 Bis-cyanoacetylhydrazone of terephthalic-aldehyde



55 Cyanoacetylhydrazone of pyruvic-aldehyde



These formulae correspond at the date of the present invention to the commonly accepted structures of these products, but are not intended to be rigorously binding.

These compounds are fully defined with regard to the practical application of the invention by the following description of their preparation. A hot aqueous solution of cyanoacetylhydrazide is mixed with a hot alcoholic solution of the compound with which the hydrazide is to be condensed. Generally, condensation takes place immediately and the condensation product precipitates in the form of crystals; if not, the solution is warmed for some time in a water bath.

The condensation of a hydrazide, and especially of cyanoacetylhydrazide, with various compounds containing a ketone or an aldehyde group is fully described in Berichte 27 (1894) 688, 40 (1907) 712 and 41 (1908) 643.

By development in a diethyl-para-phenylenediamine developer containing a color coupler according to this invention, dyestuffs are obtained with an absorption maximum at about 4,800 to 5,500 Å.

The new color couplers may be added to a developing bath containing a normal quantity of sulphite and on account of this are very stable. They may easily be produced and isolated, and are, moreover, very stable.

With aryl amine developers the new color couplers form dyestuffs practically insoluble in water and photographic baths and are characterized by an extreme brightness or brilliance. The absorption curves of these dye-stuffs are generally of marked steepness which in color photography is of great importance. Used with substituted aryl diamine developers, the color yield is generally very high.

The present invention also comprises:

(a) A new or an improved process for obtaining multi-color photographs by the use of color couplers as above described.

(b) The process for manufacturing multi-color photographs by adding the above-mentioned color couplers to the emulsion before or after it is coated and treating the latent photographic image with an aryl amine developer.

(c) New or improved color developers containing besides an aryl amine developer at least one of the above-specified color couplers.

(d) A new and improved process for color development by developing a latent photographic image with an aryl amine developer containing at least one of the aforesaid color components followed by the removal of the silver image

formed by development so that only a bright and transparent color image remains.

(e) A photographic material which contains at least in one layer a bright and transparent color image consisting of the condensation product formed during the development from a color coupler as herein described and the oxidation product of an aryl amine developer.

The aryl amine derivatives which may be used as developers are mono-, di- and tri-amino aryl compounds. As mono-amino developers may be mentioned aminophenols, aminocresols, aminonaphthols and their halogen derivatives. The most suitable and at the same time the best developers for use in the present invention are the aryl ortho- and para-diamines such as ortho- and para-phenylene diamines. These developers may be substituted in one amino group and/or in the nucleus. In this way, several developers may be obtained, as, for instance:

N-diethyl-para-phenylenediamine  
N-mono-ethyl-para-phenylenediamine  
N-dimethyl-para-phenylenediamine  
3-amino-6-diethyl-aminotoluene

These developers are usually used in the form of their salts such as hydrochlorides or sulphates.

By the expression "color development" as used in this specification is broadly to be understood the formation of a color image by the action of the color couplers as described above on any oxidizing compounds formed either during development by the action of the silver halide of the latent image on the aryl developers or by the intervention of the silver of the developed image.

In this last case, the silver image is treated with an oxidizing bath before color development.

In order to obtain color images according to the present invention, the following developing compositions may be used:

45 **Formula 1**  
N-diethyl-para-phenylenediamine-  
hydrochloride \_\_\_\_\_ grams 4  
Sodium sulphite cryst. \_\_\_\_\_ do 5  
50 Sodium carbonate cryst. \_\_\_\_\_ do 60  
Sodium hydroxide \_\_\_\_\_ do 0.5  
Water to \_\_\_\_\_ cubic centimeters 1000  
Cyanoacetylhydrazone of  
piperonal \_\_\_\_\_ grams 2  
55

**Formula 2**  
N-diethyl-para-phenylenediamine-  
hydrochloride \_\_\_\_\_ grams 4  
60 Sodium sulphite cryst. \_\_\_\_\_ do 10  
Sodium carbonate cryst. \_\_\_\_\_ do 50  
Sodium hydroxide \_\_\_\_\_ do 1  
Water to \_\_\_\_\_ cubic centimeters 1000  
Cyanoacetylhydrazone of 5-nitro-7-  
methylisatin \_\_\_\_\_ grams 2  
65

**Formula 3**  
N-diethyl-para-phenylenediamine-  
hydrochloride \_\_\_\_\_ grams 5  
70 Sodium sulphite cryst. \_\_\_\_\_ do 5  
Potassium carbonate \_\_\_\_\_ do 30  
Sodium hydroxide \_\_\_\_\_ do 1  
Water to \_\_\_\_\_ cubic centimeters 1000  
Cyanoacetylhydrazone of mono-  
bromoisoatin \_\_\_\_\_ grams 2

## Formula 4

|                                                  |                   |      |
|--------------------------------------------------|-------------------|------|
| A. N-diethyl-para-phenylenediamine-hydrochloride | grams             | 5    |
| Sodium sulphite cryst                            | do                | 5    |
| Sodium carbonate cryst                           | do                | 100  |
| Sodium hydroxide                                 | do                | 0.25 |
| Water to                                         | cubic centimeters | 1000 |
| B. Cyanoacetylhydrazone of cinnamic aldehyde     | grams             | 2    |
| Acetone                                          | cubic centimeters | 30   |

For use, B is added to A.

The color couplers may be dissolved in organic solvents, for instance acetone, though it is also possible to add them directly to the developing baths without using organic solvents.

The invention is not limited to the use of the color couplers in the photographic developing baths. One of the essential ingredients (the color coupler) which forms the dyestuff during the development may also be added to the photographic emulsion, for instance, by adsorption on the silver salts before or after the emulsion is coated. The other ingredient of the color-forming baths, especially the aryl amine developer, may afterwards be applied as a bath during the development.

The invention may be applied for the manufacture of photographic multi-color pictures on plates, paper or film provided with gelatine or any other protective colloid for silver salts. The color developing process may be carried out for developing photographic material with one or more light-sensitive layers coated on one or on both sides of the support. The silver image formed during development may easily be bleached out, whereby the bleaching bath may not exert any undesirable influence on the color image. An aqueous solution of potassium ferricyanide and sodium thiosulphate easily removes the silver without damaging the color image.

We claim:

1. A color-forming developer comprising a primary aromatic amino silver halide developing agent and as color coupler a cyanoacetylhydrazone of the general formula



wherein X represents the radical of a compound, which does not contain a group capable of coupling with the oxidation product of a primary aromatic amino silver halide developing agent to form a dye image but which is capable of forming a hydrazone by reaction with a hydrazine and selected from the group consisting of aldehydes, ketones, and compounds having two halogen atoms directly linked to the same carbon atom, and n is a positive integer selected from the group consisting of 1 and 2, the cyanoacetyl group comprising the methylene group which acts as coupling function on color development.

2. A color-forming developer comprising a primary aromatic amino silver halide developing agent and as color coupler a cyanoacetylhydrazone of the general formula



wherein X represents the radical of a compound which does not contain a group capable of coupling with the oxidation product of a primary aromatic amino silver halide developing agent to form a dye image but which is capable of forming a hydrazone by reacting with a hydrazine and selected from the group consisting

of aldehydes, ketones, and compounds having two halogen atoms directly linked to the same carbon atom, the cyano acetyl group comprising the methylene group which acts as coupling function on color development.

3. A color-forming developer comprising a primary aromatic amino silver halide developing agent and as color coupler the cyanoacetylhydrazone of piperonal.

4. A color-forming developer comprising a primary aromatic amino silver halide developing agent and as color coupler the cyanoacetylhydrazone of 5-nitro-7-methylisatin.

5. A color-forming developer comprising a primary aromatic amino silver halide developing agent and as color coupler the cyanoacetylhydrazone of cinnamic aldehyde.

6. A color-forming developer comprising a primary aromatic amino silver halide developing agent and as color coupler a di-cyanoacetylhydrazone of the general formula



wherein X represent the radical of a compound which does not contain a group capable of coupling with the oxidation product of a primary aromatic amino silver halide developing agent to form a dye image but which is capable of forming a hydrazone by reacting with a hydrazine and selected from the group consisting of aldehydes, ketones, di- and tetra-halogen compounds, the cyano acetyl group comprising the methylene group which acts as coupling function on color development.

7. A photographic emulsion containing silver halide and a color coupler consisting of a cyanoacetylhydrazone of the general formula



wherein X represents the radical of a compound, which does not contain a group capable of coupling with the oxidation product of a primary aromatic amino silver halide developing agent to form a dye image but which is capable of forming a hydrazone by reaction with a hydrazine and selected from the group consisting of aldehydes, ketones, and compounds having two halogen atoms directly linked to the same carbon atom, and n is a positive integer selected from the group consisting of 1 and 2, the cyanoacetyl group comprising the methylene group which acts as coupling function on color development.

8. A photographic emulsion containing silver halide and a color coupler consisting of a cyanoacetylhydrazone of the general formula



wherein X represents the radical of a compound which does not contain a group capable of coupling with the oxidation product of a primary aromatic amino silver halide developing agent to form a dye image but which is capable of forming a hydrazone by reacting with a hydrazine and selected from the group consisting of aldehydes, ketones and compounds having two halogen atoms directly linked to the same carbon atom, the cyano acetyl group comprising the methylene group which acts as coupling function on color development.

9. A photographic emulsion containing silver halide and a color coupler consisting of a di-cyanoacetylhydrazone of the general formula



wherein X represents the radical of a compound which does not contain a group capable of cou-

pling with the oxidation product of a primary aromatic amino silver halide developing agent to form a dye image but which is capable of forming a hydrazone by reacting with a hydrazine and selected from the group consisting of aldehydes, ketones, di- and tetra-halogen compounds, the cyano acetyl group comprising the methylene group which acts as coupling function on the color development.

10. A photographic material having at least one light-sensitive silver halide emulsion layer and containing a color coupler consisting of a cyanoacetylhydrazone of the general formula



wherein  $\text{X}$  represent the radical of a compound which does not contain a group capable of coupling with the oxidation product of a primary aromatic amino silver halide developing agent to form a dye image but which is capable of forming a hydrazone by reaction with a hydrazine and selected from the group consisting of aldehydes, ketones, and compounds having two halogen atoms directly linked to the same carbon atom, and  $n$  is a positive integer selected from the group consisting of 1 and 2, the cyanoacetyl group comprising the methylene group which acts as coupling function on color development.

11. A process for the manufacture of a colored photographic image, which comprises developing a reducible silver salt image with a color developer comprising a primary aromatic amino

silver halide developing agent and a cyanoacetylhydrazone of the general formula



5 wherein  $\text{X}$  represents the radical of a compound, which does not contain a group capable of coupling with the oxidation product of a primary aromatic amino silver halide developing agent to form a dye image but which is capable of forming a hydrazone by reaction with a hydrazine and selected from the group consisting of aldehydes, ketones, and compounds having two halogen atoms directly linked to the same carbon atom, and  $n$  is a positive integer selected from the group consisting of 1 and 2, the cyanoacetyl group comprising the methylene group which acts as coupling function on color development.

10 PIERRE JOSEPH MARIE BRUYLANTS.  
PHILIBERT LEOPOLD JOZEF  
RAYMOND MERCKX.

#### REFERENCES CITED

The following references are of record in the file of this patent:

#### UNITED STATES PATENTS

| Number    | Name      | Date          |
|-----------|-----------|---------------|
| 1,969,479 | Seymour   | Aug. 7, 1934  |
| 2,108,602 | Mannes    | Feb. 15, 1938 |
| 2,266,442 | Schinzel  | Dec. 16, 1941 |
| 2,375,344 | Braylants | May 8, 1945   |